

Patented Feb. 10, 1925.

1,525,618

# UNITED STATES PATENT OFFICE.

THEODORE NAGEL, OF BROOKLYN, NEW YORK.

## ARTIFICIAL FUEL AND METHOD OF MAKING SAME.

No Drawing.

Application filed January 2, 1923. Serial No. 610,369.

To all whom it may concern:

Be it known that I, THEODORE NAGEL, a citizen of the United States, and a resident of the borough of Brooklyn, county of 5 Kings, and city and State of New York, have invented new and useful Improvements in Artificial Fuel and Methods of Making Same, of which the following is a specification.

10 My invention relates to a process for producing artificial fuel from comminuted carbonaceous materials, examples of which are anthracite coal, coke braize, etc., and an object of my invention is the production of a 15 hard combustible water-insoluble artificial fuel in which the granules are fixed in a structure by a smokeless water-insoluble non-fusible binder.

Briefly, my invention may be realized by 20 coating the granules of comminuted carbonaceous material with a binding material, such as acidulated syrup, acidulated syrup and phosphoric acid, causticized vegetable glue and syrup, sulphite pitch and phosphoric acid, etc., which, upon heating and cooling is converted into a hard combustible water-insoluble non-fusible binder. The mixture is then pressed to exclude the voids 25 thereof to force the granules of the comminuted material into intimate contact and finally heated and cooled to convert the binding material into a binder which is combustible water-insoluble and non-fusible and is substantially smokeless and odorless when burning. This binder surrounds 30 the granules of the carbonaceous material and fixes them in a water-insoluble structure, that is a structure which though not necessarily waterproof will not soften and disintegrate in water and does not disintegrate 35 while burning, that is, does not soften or flow.

In practising my invention I prefer to use black strap molasses—the residue after 40 extracting the sugar crystals from cane juice at sugar cane mills or the residue syrup from sugar refineries and when phosphoric acid is used I prefer a solution of phosphoric acid.

45 50 A specific manner of practising my invention is as follows:

The carbonaceous material is first of all reduced or comminuted to from  $\frac{3}{2}$  of an inch in diameter to 200 mesh. This material may be treated either moist or dry. I then preferably, though not necessarily, dry

and heat this comminuted material to a temperature not to exceed substantially 400° F. and to this material add a binding material such as for example, the above referred to acidulated syrup and a solution of phosphoric acid, the amount of syrup not to exceed substantially 7½% by weight of the comminuted material and the amount of acid not to exceed 1½%  $H_3PO_4$  by weight of the comminuted material.

The carbonaceous material and the binder are thoroughly mixed so as to coat or cover substantially all of the granules of the material. The mixture is then pressed, in a 70 briquet press for example, to exclude the voids of the mixture and to force the granules thereof into intimate contact, then this pressed mixture is heated to a temperature substantially not in excess of 800° F. and 75 subsequently cooled. The heating and subsequent cooling of the mixture converts the binding material into a combustible water-insoluble non-fusible binder which fixes the granules of the mixture in a water-insoluble 80 structure that burns without softening and flowing. In the heating of the mixture a chemical reaction takes place forming phosphates.

It is to be understood that the expression 85 "non-fusible" binder used throughout this description and the accompanying claims is to be interpreted to mean a binder which does not fuse at the burning temperature of the carbonaceous material employed in making up the fuel.

It is to be also understood that, while I have specifically referred to various binding materials as suitable for use in the practice 90 of my improved process these materials are merely illustrative, and that binding materials other than those specifically referred to may be used, the desideratum being a hard water-insoluble structure, the granules of which are fixed therein by a binder which 95 upon heating and cooling is converted into a binder that is non-fusible and water-insoluble and emits substantially no smoke or odor while burning.

It will be obvious to those skilled in this 100 art that my improved method produces an artificial fuel composed of comminuted carbonaceous material, the granules of which are fixed in a hard water-insoluble structure by a binder which is non-fusible and water-insoluble. The binder being non-fusible at 105 the burning temperature of the carbona-

ceous material holds the granules of the fuel to the structure while the granules are burning, thereby preventing softening and flowing of the structure.

5 I claim:

1. The process of making artificial fuel which process consists in mixing with comminuted carbonaceous material a binding material which, upon heating and cooling is converted into a non-fusible binder, pressing the mixture to bring the granules thereof into intimate contact, and subsequently fixing the granules of the carbonaceous material in a structure by heating and cooling 10 the mixture to convert the binding material into a non-fusible binder.

2. The process of making artificial fuel which process consists in mixing with comminuted carbonaceous material a binding material which, upon heating and cooling 20 is converted into a water-insoluble, non-fusible binder, subjecting the mixture to pressure to bring the granules thereof into intimate contact and subsequently fixing the 25 granules of the carbonaceous material in a water-insoluble structure by heating and cooling the mixture to convert the binding material into a water-insoluble non-fusible binder.

30 3. As an article of manufacture, an artificial fuel composed of comminuted carbonaceous material and a binder containing phosphorus.

4. As an article of manufacture, an artificial fuel composed of comminuted carbonaceous material and added phosphoric acid.

40 5. As an article of manufacture, an artificial fuel composed of comminuted carbonaceous material and salts of phosphorus.

6. As an article of manufacture, an artificial fuel composed of comminuted carbonaceous material and phosphates.

7. As an article of manufacture, an ar-

tificial fuel composed of comminuted carbonaceous material and a binder containing organic carbon and phosphates.

8. The process of making artificial fuel which process consists in mixing with comminuted carbonaceous material a binding material which, upon heating is converted 45 into a non-fusible binder, pressing the mixture to bring the granules thereof into intimate contact, and subsequently fixing the granules of the carbonaceous material in a 50 structure by heating the mixture to convert the binding material into a non-fusible binder.

9. A briquette comprising comminuted material and a phosphoric acid binding material, said mixed materials being indurated 60 by heating.

10. The method of making fuel briquettes which comprises subjecting suitable comminuted material to the action of a phosphoric acid, moulding the material into the desired shape, and heating the material at a temperature above about 200° C. until the material acquires the desired hardness.

11. A briquet comprising a heat-indurated 70 mass of commingled material and a phosphoric acid binding material.

12. The method of making briquets which comprises subjecting comminuted material to the action of a phosphoric acid, molding 75 the material into briquettes of any desired shape and indurating the briquets by the action of heat.

13. A fuel briquet comprising comminuted carbon and a phosphoric acid binding 80 material.

14. A fuel briquet comprising anthracite coal culm and a phosphoric acid binding material.

This specification signed this 30th day of December, 1922.

THEODORE NAGEL.